

## [54] PROCESSES FOR THE MANUFACTURE OF SLUB EFFECT YARNS

[75] Inventor: William Wilson, Pontypool, England

[73] Assignee: Imperial Chemical Industries Limited, London, England

[22] Filed: May 29, 1973

[21] Appl. No.: 364,634

## [30] Foreign Application Priority Data

June 5, 1972 Great Britain ..... 26135/72

[52] U.S. Cl. .... 57/157 F, 57/34 B, 28/72.12

[51] Int. Cl. .... D02g 3/02, D01h 1/00

[58] Field of Search ..... 57/34 R, 34 B, 144, 157 R, 57/157 F, 160; 28/72.12

## [56] References Cited

## UNITED STATES PATENTS

3,116,589 1/1964 Edwards et al. .... 57/157 F

|           |         |                       |            |
|-----------|---------|-----------------------|------------|
| 3,473,315 | 10/1969 | LeNoir .....          | 57/157 F X |
| 3,474,613 | 10/1969 | Joarder et al. ....   | 57/34 B    |
| 3,517,498 | 6/1970  | Burellier et al. .... | 57/34 B X  |

Primary Examiner—Donald E. Watkins  
 Attorney, Agent, or Firm—Cushman, Darby & Cushman

## [57] ABSTRACT

A method for the preparation of a tension stable slub effect yarn, wherein a core yarn at zero overfeed is fed into a turbulence chamber and an effect yarn is simultaneously injected into the turbulence chamber at 100-120 percent overfeed and permitted to combine with the core yarn and the combined yarn is then intermingled and wound-up.

## 10 Claims, 1 Drawing Figure



PATENTED MAY 28 1974

3,812,668



## PROCESSES FOR THE MANUFACTURE OF SLUB EFFECT YARNS

The present invention relates to an improved method for the manufacture of a slub effect yarn and to yarn produced by the process. It is known that a slub effect yarn can be manufactured from two continuous filament yarns by methods involving combining the yarns in the vicinity of an air jet under turbulent conditions, one of the said yarns being fed at a greater rate than the other to form slub-like collections of filaments of the one yarn along the length of the other.

Thus, in British Patent Specification No. 1,239,758 there is described a process in which one end of yarn is positively overfed to an intermingling jet and a second yarn is fed to the same jet without positive feed to yield an intermingled combined yarn in which the overfed component forms slub effects along the length of the yarn.

In British Patent Specification No. 1,036,151 a yarn which is required to be bulked is drawn through a turbulence chamber into which a gas is injected in a direction opposite to that in which the yarn is being forwarded. It is also disclosed that a second yarn under tension may be drawn through the same chamber to act as a carrier for the bulked yarn to yield a slub effect combined yarn.

We have now found that a tension stable slub effect yarn can be obtained by supplying a first core yarn to a turbulence chamber, having yarn inlet and exit passage ways, under conditions of zero overfeed so that no bulk is inserted into the yarn, and injecting a second effect yarn under conditions of overfeed by the action of a fluid jet, the fluid being permitted to exhaust out of the inlet and exit passage ways of the turbulence chamber, the combined yarn from the turbulence chamber then being forwarded through an intermingling jet and finally wound up in the form of a coherent slub effect yarn.

By injecting the effect yarn into the turbulence chamber under conditions of positive overfeed, by means of a fluid jet, the effect yarn becomes looped and entangled and at random intervals becomes attached in the form of balls to the core yarn and is withdrawn with the core yarn from the turbulence chamber. The intermingling jet then firmly locks the effect yarn into the core yarn to yield the cohered random slub effect yarn.

The effect yarn may be overfed into the turbulence chamber at a rate of about 60 - 120 percent. To achieve maximum benefit from the process, the effect yarn may be overfed at a rate of about 100-120 percent.

The core yarn may be positively fed into the turbulence chamber through a pair of nip or feed rolls. Alternatively it may be withdrawn from a supply package by the tension imparted by the wind-up apparatus and, optionally, a yarn tension device may be employed above the turbulence chamber to assist in maintaining sufficient tension in the yarn to avoid bulking.

It is preferred that the exit passageway of the turbulence chamber is of smaller diameter than the inlet passageway. The inlet passageway may be restricted by a cap or baffle at the entrance to confine yarn and fluid movement which could adversely affect the stability of the incoming core yarn.

It is also preferred that the effect yarn is injected into the turbulence chamber near to the junction of the inlet

and exit passageways. The effect yarn is preferably injected into the turbulence chamber in a direction perpendicular or substantially perpendicular to the forwarding direction of the core yarn.

5 The nature of the slub effect yarn is affected by the positioning of the intermingler jet, the air pressure therein and in particular by the angle between the axis of the intermingler yarn passageway and the axis of the turbulence chamber yarn passageway. Increasing the 10 amount of air exhausting from the intermingling jet and entering the outlet passageway of the turbulence chamber, i.e., decreasing the above angle, produces long thin slubs; decreasing the amount of air by increasing the angle produces short thick slubs. The nature of the slub 15 effect yarn is also affected by the nature of the effect yarn and the extent of overfeed of said effect yarn.

In a preferred embodiment of the invention, the angle between the yarn emerging from the intermingler jet and the axis of the intermingler yarn passageway is 20 at least 50°.

There is no limitation on the type of yarn which may be employed for either the feed yarn or the core yarn. Yarns of, for example, polyester, polyamide, rayon, acetate or acrylics may be employed as may yarns of naturally occurring fibres such as wool, cotton, etc. The 25 yarns may be bulked yarns, staple yarns or continuous filament yarns.

The invention will now be more fully described with reference to the drawing filed with the provisional specification.

In the drawing the core yarn 1 is withdrawn from the package 2 and passes through guide 3 into the turbulence chamber 4. The turbulence chamber has a core inlet passage way 5 and an outlet passage way 6. The inlet passageway may be of cylindrical, conical or square cross-section. It may be baffled or unbaffled and may be open or restricted at the entrance. The passage way has a step 7 (but this is not essential) such that the outlet passageway is of smaller diameter than the inlet passage way. Below the turbulence chamber is an intermingler 8, a free running roller 9 and a guide 10 which is located above a conventional wind-up apparatus, not shown. An effect yarn package 12, carrying effect yarn 11 is mounted opposite to the turbulence chamber 4 together with a guide 13 and an air disperser 14. In a preferred embodiment of the invention, the effect yarn is positively fed to the air disperser through a pair of nip or feed rolls.

50 Optionally, a pair of feed rolls 15, 16 may be located between the core yarn package and the turbulence chamber. A steam heater 17 may be situated between the free running roller and the wind-up to give loop deformation and change the tactile properties of the yarn.

55 The following Examples illustrate but do not limit the invention.

### EXAMPLE 1

Using the apparatus as illustrated in the drawing, a 60 167 dtex, 30 filament polyester core yarn was passed through the turbulence chamber to the wind-up at a speed of 500 ft/min and a 78 dtex, 20 filament nylon 66 effect yarn was injected through the air disperser 14 into the turbulence chamber 4 at an air pressure of 65 10-20 p.s.i. The nylon 66 effect yarn was injected into the chamber at an overfeed of 100-120 percent. The effect yarn formed loops and at random intervals at-

tached itself to the core yarn and the combined core and effect yarn then passed through the intermingler jet 8 around the free running roller to the wind-up.

### EXAMPLE 2

The apparatus as illustrated in the drawing was used except that the effect yarn was positively fed to the air disperser 14 by a nip roll system with the disperser situated to inject the effect yarn into the upper portion of the turbulence chamber exit passageway and the pair of nip rolls 15, 16 was omitted. The process conditions were as follows:

Core yarn: 110 dexitex/48 filament poly(ethylene terephthalate) yarn

Effect yarn: 84 decitex/36 filament poly(ethylene terephthalate) yarn

Wind-up speed: 1100 ft/min

Overfeed of effect yarn: 115-125%

Air pressure to disperser: 5-10 p.s.i.

Air pressure to intermingler: 70-80 p.s.i.

Angle between axis of intermingler yarn passageway and axis of turbulence chamber yarn passageway: 16°-17°

The slab effect yarn so produced had a decitex of 245 and contained 45 and 55 wt percent of core and effect yarns respectively. A 1,000 metre length of the slab effect yarn contained 4,194 slubs of which 56 percent were of length between 1 to 2 cm, 37 percent were of length between 2 to 5 cm and 7 percent were of length between 5 to 10 cm. The slab effect yarn was particularly suitable for weft knitting outlets.

### EXAMPLE 3

Example 2 was repeated except that the angle between the axis of the intermingler yarn passageway and the axis of the turbulence chamber yarn passageway was 12°-15°.

A 1,000 metre length of the slab effect yarn so produced contained 660 slubs of length distribution:

17% between 1 to 2 cm

21% between 2 to 5 cm

19% between 5 to 10 cm

21% between 10 to 20 cm

19% between 20 to 40 cm

3% above 40 cm

The slab effect yarn was particularly suitable for

weaving outlets.

What I claim is:

1. A process for producing a tension stable slab effect yarn which comprises supplying a first core yarn to a turbulence chamber, having yarn inlet and exit passage ways, under conditions of zero overfeed so that no bulk is inserted into the yarn, and injecting a second effect yarn under conditions of overfeed by the action of a fluid jet, the fluid being permitted to exhaust out of the inlet and exit passage ways of the turbulence chamber, the combined yarn from the turbulence chamber then being forwarded through an intermingling jet and finally wound up in the form of a coherent slab effect yarn.
- 15 2. A process according to claim 1 in which the angle between the yarn emerging from the intermingler jet and the axis of the intermingler yarn passageway is at least 50°.
- 20 3. A process according to claim 1 in which the exit passageway of the turbulence chamber is of smaller diameter than the inlet passageway.
- 25 4. A process according to claim 1 in which the effect yarn is injected into the turbulence chamber near to the junction of the inlet and exit passageways.
- 30 5. A process according to claim 1 in which the angle between the axis of the intermingler yarn passageway and the axis of the turbulence chamber yarn passageway is such as to allow some of the air exhausting from the intermingler jet to enter the outlet passageway of the turbulence chamber.
- 35 6. A process according to claim 1 in which the effect yarn is overfed into the turbulence chamber at a rate of 60-120 percent.
7. A process according to claim 1 in which the effect yarn is positively fed to the fluid jet.
- 35 8. A process according to claim 1 in which the effect yarn is injected into the turbulence chamber in a direction perpendicular or substantially perpendicular to the 40 forwarding direction of the core yarn.
9. A process according to claim 1 in which the core yarn is positively fed into the turbulence chamber.
- 45 10. A process according to claim 1 in which the slab effect yarn is heated between the intermingler jet and the wind-up.

\* \* \* \* \*